

Dec. 29, 1925.

1,567,791

E. DUHME

ELECTROLYTIC PRODUCTION OF METALS

Filed Nov. 1, 1924



Inventor  
Emil Leuhme  
by Knight Br. *Attorney*

## UNITED STATES PATENT OFFICE.

EMIL DUHME, OF BERLIN-CHARLOTTENBURG, GERMANY, ASSIGNOR TO SIEMENS & HALSKE, AKTIENGESELLSCHAFT, OF SIEMENSSTADT, NEAR BERLIN, A CORPORATION OF GERMANY.

## ELECTROLYTIC PRODUCTION OF METALS.

Application filed November 1, 1924. Serial No. 747,366.

*To all whom it may concern:*

Be it known that I, EMIL DUHME, a citizen of the German Empire, residing at Berlin-Charlottenburg, Germany, have invented <sup>5</sup> certain new and useful Improvements in the Electrolytic Production of Metals, of which the following is a specification.

My invention relates to improvements in the electrolytic production of metals.

<sup>10</sup> The hitherto employed processes for electrolytically producing metals show the drawback that the impurities of the anode material are deposited or precipitated on the cathode together with the metal so that <sup>15</sup> the product of the process is a metal which contains a certain amount of impurities.

<sup>20</sup> The object of my invention is a process and apparatus in which the impurities of the anode material are kept away from the cathode so that the product obtained is a refined or almost pure metal.

<sup>25</sup> The invention is based on the recognition that by electrolytically depositing metal on a plurality of cathodes, deposits of different degrees of purity or refinement can be obtained if the individual cathodes are differently disposed relatively to the anode either electrically or with regard to distance. The difference in the composition of

<sup>30</sup> the deposits obtained on the several cathodes resides in the fact that the transition of the metal from the anode to the cathode is a purely electrical process, whereas the transition of the impurities from the anode <sup>35</sup> to the cathode is an almost exclusively chemical process.

<sup>40</sup> Thus, according to the present invention, even if only two cathodes are employed, of which for instance, one is disposed at a smaller distance from the anode than the other, deposits of different degrees of purity may be obtained on these cathodes. It is true that in such cases a considerable percentage of the metal to be purified will be <sup>45</sup> deposited at the nearer cathode, but a by far greater percentage of impurities will likewise be deposited on this nearer cathode. I shall designate in the following description the cathode on which the greater percentage <sup>50</sup> of impurities are deposited, as auxiliary cathode and the other cathode on which the

refined desired metal is deposited, the main cathode.

The effect referred to hereinbefore results from the diffusion of the impurities contained in the metals through the electrolyte, and thus the concentration of the impurities will be the smaller, the greater the distance is between the cathode and the anode. Besides the impurities contained in the metals <sup>55</sup> to be refined are largely of a nature, electrically, such that they have a greater tendency to deposit than the metals to be refined, and therefore they will deposit to a very large extent at the nearer cathode, i. e., <sup>60</sup> the auxiliary cathode. By thus repeating the process just described, the initially small difference in purity of the deposited metal at the two cathodes may gradually be increased. <sup>65</sup>

<sup>70</sup> This difference in composition of the deposits at different distances of the cathodes from the anode can be considerably increased by making the auxiliary cathode of smaller area than the more remote or main cathode. This will result in a greater portion of the desired metal traveling to the main cathode, while at the same time the difference in surface between the two cathodes <sup>75</sup> has no effect with regard to the deposition of impurities.

<sup>80</sup> It is desirable to deposit on the auxiliary cathode, whose deposits largely are to consist of impurities, only so much of the desired metal as is necessary for binding the impurities. For this purpose, according to the invention, also the electrolytical relation of the two cathodes to the anode is made different. This is accomplished according to the invention for instance, by permitting a current of smaller intensity to flow between the anode and the auxiliary cathode than between the anode and the main cathode. The effect attained thereby may be further increased by permitting an alternating current to flow between the anode and the auxiliary cathode, whose maximum potential is greater <sup>85</sup> than the direct current potential which is effective between the electrodes.

<sup>90</sup> In order to deposit on the auxiliary cathode aside from the impurities only as much metal as is necessary for binding the impurities, the direct current flowing be-

tween the anode and the auxiliary cathode—  
aside from the alternating current flowing  
therebetween—is made correspondingly  
smaller in intensity. This decrease in di-  
rect current may be attained for instance by  
inserting a resistance between the auxiliary  
cathode and the negative pole of the direct  
current source. Thus an “unsymmetrical  
alternating current,” as it were, flows be-  
tween the anode and the auxiliary cathode.  
The effect obtained thereby is essentially as  
follows:

The alternating current which flows be-  
tween the anode and the auxiliary cathode  
prevents a deposit of the desired metal on  
the auxiliary cathode. However, since,  
aside from the alternating current also di-  
rect current of small intensity flows be-  
tween the auxiliary cathode and the anode, a  
small percentage of the desired metal is de-  
posited on the auxiliary cathode by means  
of this small direct current. This small  
amount of metal deposit is sufficient to bind  
the impurities which diffuse through the  
electrolyte and which are deposited on the  
auxiliary cathode so that only a very small  
percentage of these impurities travels to the  
main cathode in whose vicinity the concen-  
tration of the impurities in the electrolyte  
is very much smaller than in the vicinity of  
the auxiliary cathode. The strong direct  
current which flows between the anode and  
the main cathode now causes the deposition  
of the metal on the main cathode except  
the small portion of metal which remains on  
the auxiliary cathode on account of the al-  
ternating current flowing.

In the drawing affixed to this specification  
and forming part thereof an apparatus is  
illustrated which is adapted to carry out  
the above described process for obtaining re-  
fined metals and more particularly for ob-  
taining iron free from phosphorus.

Referring to this drawing, 1 is a vessel  
or tank containing the electrolyte, 2 a cylin-  
drical anode, 3 the main cathode and 4 the  
auxiliary cathode. This auxiliary cathode 4  
is cylindrical and perforated. In the inter-  
ior of the auxiliary cathode 4 is located the  
main cathode 3. The anode 2 and the main  
cathode 3 are directly connected with the  
source of continuous current 5, the auxiliary  
cathode 4 being connected with the negative  
pole of the source of continuous current  
across a resistance 6. Between anode and  
auxiliary cathode 4 there is, furthermore,  
connected a source 7 of alternating current  
which gives satisfactory results at the usual  
frequency of, for instance, 40 to 50 cycles.

The action of this improved process is  
probably based on the fact that those phases  
of the alternating current during which the  
electrode 4 becomes anode and the electrode  
2 cathode increase the concentration of the  
impurities, for instance, the phosphorus com-

bination, because under the influence of  
electrolysis these combinations travel to the  
anode for the time being. The subsequently  
reversed direction of the current brought  
about by the alternation of the current makes 70  
the electrode 4 into a cathode. The hydro-  
gen in its nascent state generated at the aux-  
iliary cathode besides the iron deposit re-  
duces the previously accumulated phos-  
phorus combinations. The liberated phos-  
phorus combines at the auxiliary cathode  
with the iron into iron phosphide. The iron  
at the anode 2 serving for the production of  
the solution passes to the main cathode 3  
where it is deposited in almost pure state. 80  
Experiments have shown that the contents of  
phosphorus of the iron deposited on the  
main cathode may by means of the improved  
process be reduced to less than one thou-  
sandth of the phosphorus previously con-  
tained in the anode. 85

What I claim as my invention is:—

1. A process for electrolytically depositing  
metals substantially free from impuri-  
ties on a cathode, consisting in maintaining  
an auxiliary cathode nearer the anode than  
the main cathode on which latter the desired  
pure metal is to be deposited and in supply-  
ing a suitable current to said auxiliary cath-  
ode and said anode, causing a comparatively  
small but desired metal deposit on the aux-  
iliary cathode, whereby, due to larger concen-  
tration of the impurities near the anode,  
they are deposited on the auxiliary cathode  
to a greater extent than on the more remote 100  
main cathode. 95

2. A process for electrolytically depositing  
metals substantially free from impurities  
on a cathode, consisting in maintaining an  
auxiliary cathode nearer the anode and of  
smaller area than the main cathode on which  
latter the desired pure metal is to be de-  
posited and in supplying a suitable current  
to said auxiliary cathode and said anode,  
whereby due to the larger main cathode area  
a greater portion of the desired metal is de-  
posited on the main cathode. 105

3. A process for electrolytically depositing  
metals substantially free from impuri-  
ties on a cathode, consisting in maintaining  
an auxiliary cathode nearer the anode than  
the main cathode on which latter the desired  
pure metal is to be deposited, and in supply-  
ing an unsymmetrical alternating current to  
said auxiliary cathode and said anode, caus-  
ing a comparatively small but desired metal  
deposit on the auxiliary cathode, sufficient  
to bind the impurities deposited thereon,  
whereby due to larger concentration of the  
impurities near the anode, they are deposited  
on the auxiliary cathode to a greater extent  
than on the more remote main cathode. 115

4. A process for electrolytically deposit-  
ing metals substantially free from impuri-  
ties on a cathode, consisting in maintaining 120  
125  
130

an auxiliary cathode nearer the anode than the main cathode on which latter the desired pure metal is to be deposited and in supplying direct current of suitable voltage to said anode and main cathode, and in supplying to said anode and auxiliary cathode alternating current of suitable voltage and also direct current of lower voltage than the

voltage of the current supplied to the main cathode, whereby due to larger concentration of the impurities near the anode, they are deposited on the auxiliary cathode to a greater extent than on the more remote main cathode. 10

In testimony whereof I affix my signature.  
EMIL DUHME.